

# UNITED STATES PATENT OFFICE.

VICTOR FUSSGÄNGER, OF HÖCHST-ON-THE-MAIN, GERMANY, ASSIGNOR TO  
FARBWERKE, VORM. MEISTER, LUCIUS & BRÜNING, OF HÖCHST-ON-THE-  
MAIN, GERMANY, A CORPORATION OF GERMANY.

## BLUE FIBROUS MATERIAL AND PROCESS OF DYEING SAME.

No. 816,457.

Specification of Letters Patent.

Patented March 27, 1906.

Application filed February 7, 1905. Serial No. 244,639.

To all whom it may concern:

Be it known that I, VICTOR FUSSGÄNGER, Ph. D., chemist, a citizen of the Empire of Austria-Hungary, residing at Höchst-on-the-  
Main, Germany, have invented certain new  
and useful Improvements in the Processes of  
Dyeing Blue, of which the following is a  
specification.

I have found that by oxidizing a mixture  
of alkylated diamidobenzhydrols and para-  
oxy or para-amido diphenylamin and their  
derivatives new dyestuffs of a vivid blue may  
be obtained which are distinguished by their  
fastness to washing, soap, soda, alkali, and  
acid even in the absence of a tannin mordant.

It is known that tetramethyldiamidoben-  
zhydrol with acids yields beautifully blue  
tinted salts decolorized by an excess of acid.  
On tannin-mordanted cotton or silk these  
salts produce beautiful shades, lacking fast-  
ness, however, and being readily decom-  
posed by soap, dilute alkalies, or acids.  
(Compare Nietzki, *Chem. Organ. Farbstoffe*,  
III edition, pages 110, 111.) The new dy-  
estuffs obtained by this process, therefore,  
must not be mistaken for the known salts of  
the alkylated diamidobenzhydrols, as it is a  
question here of new condensation products.

If tetramethyldiamidobenzhydrol alone is  
oxidized, no dyestuff is obtained, but by ox-  
idizing para-oxy or para-amido diphenylamin  
by itself a light gray is produced. If, how-  
ever, the hydrol be mixed with one of these  
diphenylamin derivatives in a printing or pad-  
ding color and oxidized on the fiber, new dye-  
stuffs of beautiful shades and excellent fast-  
ness are obtained. In a similar manner react  
the derivatives of para-oxy or para-amido  
diphenylamin—like, for instance, para-amido-  
para-oxy-diphenylamin, para-diamidodiphe-  
nylamin and their homologues with tetra-  
methyldiamidobenzhydrol and other alka-  
lylated diamidobenzhydrols. The correspond-  
ing methane derivatives, like tetramethyldi-  
amidodiphenylmethane, when oxidized on  
the fiber together with para-amidodiphenyl-  
amin also yield a blue dyestuff of the same  
excellent properties. This is due probably  
to the hydrol being first formed from the  
methane derivative, whereupon it reacts  
with para-amidodiphenylamin. Thus, for in-  
stance, para-oxydiphenylamin and tetra-  
methyldiamidobenzhydrol yield a vivid vio-

let-blue. Para-oxydiphenylamin and tetra-  
ethyldiamidobenzhydrol yield a blue. Para-  
amidodiphenylamin and tetramethyldiami-  
dobenzhydrol yield a marine blue. Para-  
amidodiphenylamin and tetraethylamido-  
benzhydrol yield a greenish blue. Para-  
amidodiphenylamin and tetramethylamido-  
diphenyl-methane yield a dark blue. Para-  
amidodiphenylamin and tetraethylamido-  
diphenyl-methane yield a greenish blue.  
Para-amidomethyl-diphenylamin and tetra-  
methyldiamidobenzhydrol yield a blue. Para-  
amidophenyltolylamin and tetramethyldi-  
amidobenzhydrol yield a blue. Para-amido-  
para-oxydiphenylamin and tetramethyldi-  
amidobenzhydrol yield a dark blue. Phenyl-  
para-amidodiphenylamin and tetramethyl-  
diamidobenzhydrol yield a blue. Para-di-  
amidophenylamin and tetramethyldiamido-  
benzhydrol yield a dark blue. Dimethyl-  
para-amido-para-oxyphenyltolylamin and  
tetramethyldiamidobenzhydrol yield a blue.

The dyestuff obtained from tetraethylamido-  
benzhydrol with para-oxydiphenylamin  
is especially fast to soap and soda.

The shades of the dyestuffs obtained with  
para-oxydiphenylamin are essentially purer  
and more vivid than those obtained with para-  
amidodiphenylamin, but to become faster to  
acids require a slight addition of tannin.

The present application has in common  
with the application on which Letters Pat-  
ent were issued on August 8, 1905, No.  
796,715, a partial application of para-amido-  
diphenylamin and its derivatives, but is dis-  
tinguished from it by using alkylated di-  
amidobenzhydrols as one of the components.  
Moreover, in the cited application quinone-  
imid dyestuffs are formed on the fiber, where-  
as here new triphenylmethane dyestuffs may  
be obtained. Besides the fastness to soap  
and soda of the dyestuffs obtained by this  
process is greater and the shades are more  
vivid than the products of the application  
referred to.

The two bodies to be condensed are mixed  
in a printing or padding color with the requi-  
site solvent and thickening agent, whereupon  
oxidizing agents are added and the whole ap-  
plied to the vegetable or animal fiber. It is  
developed by drying or subsequent steaming.  
No free mineral acid is necessary, the oxida-  
tion taking place with organic salts and

chlorates. This prevents the fiber from being attacked.

The process may be modified with para-oxydiphenylamin by applying the different components successively and by oxidizing them together or by separately preparing the leuco compound from hydroxyl and the diphenylamin derivative. It is then applied to the fiber and oxidized by steaming with chlorates or other oxidizing agents, such as potassium bichromate.

### Example 1.

89 grams of *4*-nitrophenylmethylbenzylalcohol of nitro-para-cum are dissolved on the water bath with:

19 grams of *p,p'*-oxydiphenylamine,  
100 cubic centimeters of acetic acid, of 6% per cent.,  
30 cubic centimeters of *cro*-acid of fifty per cent, stirred into

76 grams of acid-starch thickening, adding:

10 grams of chlorins of sodium,  
33 cubic centimeters of water,  
16 cubic centimeters of aluminum chlorid of twenty per cent.,

5 cubic centimeters of *cro*-chlorid of twenty per cent.,  
195 cubic centimeters of water.

1 kilogram.

### Example 13:

13 grains of commercial tetramethylidismidobenzhydrol and  
15 grains of  $\alpha$ -naphthalidophenylphosphine are heated with  
300 cubic centimeters of acetic acid of 6° Beamsé specific  
gravity and  
20 cubic centimeters of lactic acid of fifty per cent. and  
added into  
300 grams of acetate of starch thickening.  
14 grams of chlorate of sodium,  
26 cubic centimeters of water,  
15 cubic centimeters of aluminum chloride of 20° Beamsé  
specific gravity,  
40 cubic centimeters of casein-chlorid of twenty per cent. and  
170 cubic centimeters of water being added

The printed fabric is dried and steamed for a short time in the Mather-Platt apparatus or 35 for one hour in a vessel without pressure, then washed and soaped.

*Example III.*

40      20 grams of tetramethylidiaminobenzhydrol of about ninety per cent,  
 10 grams of para-oxydiphenylamin,  
 100 cubic centimeters of acetic acid of 8° Baumé specific gravity,  
 50 cubic centimeters of lactic acid of fifty per cent,  
 900 grams of acid-starch thickening,  
 10 grams of tartric acid,  
 6 cubic centimeters of cero-chlorid of 43° Baumé specific gravity,  
 150 cubic centimeters of water,  
 10 grams of chlorate of sodium,  
 20 cubic centimeters of water,  
 20 grams of tanin,  
 20 cubic centimeters of water.

45      1 kilogram.

50 The fabric is printed, steamed in the Mather-  
Platt or in a closed vessel, passed through an  
antimony-bath, washed, soaped, and dried.

#### Example IV.

The fabric is printed, dried, passed through a bath of five grams of potassium bichromate and three grams of sulfuric acid to the liter at about 60° centigrade, washed, and soaped. 60

### Example V.

65

A 15 grams of commercial tetraarnethylamido benzhydrol and  
 11 grams of para-aminodiphenylamin are dissolved in  
 100 cubic centimeters of acetic acid of fifty per cent, and  
 20 cubic centimeters of lactic acid of fifty per cent and  
 stirred into  
 100 grams of tragacanth water, sixty grams to the liter,  
 200 cubic centimeters of water,  
 70

B 14 grams of chlorate of sodium,  
 23 cubic centimeters of water,  
 18 cubic centimeters of aluminium chlorid of 30° Baumé  
 specific gravity,  
 10 cubic centimeters of cero-chlorid of twenty per cent.,  
 400 cubic centimeters of water. Before use, pour color  
 B into A and make up to 750 cc.

The fabric is padded, dried, and the blue developed by steaming for a short time or on the drying-cylinder or in the oxidation-chamber.

The process may be applied to vegetable or animal fibers, but with woolly material the reducing power of the fiber has to be considered, which requires greater quantities of 85 chlorate or chlorinated or acidified woolstuffs.

Resist effects may be obtained in the usual manner by reducing agents, such as tin salt, potassium sulfite, hydrosulfite, and the like.

Having now described my invention, what I claim is—

1. The process herein described for the manufacture of fast-blue dyestuffs on the fiber, which consists in saturating the fiber with a mixture of alkylated diamidobenzhydrols and diphenylamin derivatives and in oxidizing same together by means of an oxidizing agent. 95

2. The process of dyeing, which consists in preparing leuc compounds from a mixture of alkylated diamidobenzhydrols and diphenylamin derivatives, saturating the fibers with said compounds and oxidizing them to a dye by oxidizing agents.

3. As a new product, a fibrous material of blue shade, obtained by oxidizing a mixture of alkylated diamidebenzhydrols and diphenylamin derivatives within the fiber, being fast to water, soap, soda, dilute alkalies and acids and reduced by hydrosulfite. 111

In testimony that I claim the foregoing as my invention I have signed my name in presence of two subscribing witnesses.

## VICEDOR. FUSSGÄNGER.

Witnesses.

ALFRED BRISBOIS,  
BERNHARD LYBECKER.